

Oct. 17, 1944.

R. J. AUST

2,360,312

METHOD OF MAKING INSULATED WIRE UNITS

Filed July 10, 1941

Fig. 1



Fig. 3



Fig. 2



Fig. 4



Fig. 5



Fig. 6



INVENTOR  
Robert J. Aust  
By *Paul Robbin*  
ATTORNEY

BY

## UNITED STATES PATENT OFFICE

2,360,312

## METHOD OF MAKING INSULATED WIRE UNITS

Robert J. Aust, Indianapolis, Ind., assignor to  
P. R. Mallory & Co., Inc., Indianapolis, Ind., a  
corporation of Delaware

Application July 10, 1941, Serial No. 401,725

2 Claims. (Cl. 154—2.21)

This invention relates to an insulated wire unit and method of making the same.

An object of the invention is to improve insulated wire units and their method of manufacture.

Other objects of the invention will be apparent from the following description and accompanying drawing taken in connection with the appended claims.

The invention comprises the features of construction, combination of elements, arrangement of parts, and methods of manufacture and operation referred to above or which will be brought out and exemplified in the disclosure hereinafter set forth, including the illustrations in the drawing.

In the drawing:

Figure 1 illustrates a length of insulated wire used in the manufacture of a wire unit of the present invention;

Figure 2 illustrates a step in the process of making the wire unit;

Figure 3 illustrates a modified method which may be substituted for that shown in Figure 2;

Figure 4 illustrates a unit in semi-completed condition; and

Figures 5 and 6 illustrate two types of wire units in completed condition.

In various types of electrical apparatus it is necessary to use relatively short lengths of insulated wire to electrically connect various terminals of the apparatus. For example, in electromagnetic vibratory interrupters such as are used in power supply systems and radio receiving sets and the like relatively short lengths of braided copper wire insulated with a suitable insulating sleeve are needed to connect the electromagnet and the various contact springs which are located inside a suitable can or container with terminals mounted in or projecting from one wall or end of the container.

In the past it has been customary to use a flexible stranded or braided copper wire which was cut to the desired length, tinned at its ends and then covered with a pre-cut length of rubber tubing for insulation purposes. This arrangement has proved unsatisfactory in many cases due to the fact that relatively high operating temperatures are sometimes encountered in the vibrators and the rubber tubing is subjected to melting and to oxidation hardening in service resulting in insulation failures and other troubles. This method of making an insulated lead wire has also required several operations and been somewhat expensive.

A feature of the present invention resides in the use of a wire which is insulated with a braided

or woven fibre covering, the fibres of which are thermoplastic or thermoadhesive in nature.

While a preferred embodiment of the invention is described herein, it is contemplated that considerable variation may be made in the method of procedure and the construction of parts without departing from the spirit of the invention. In the following description and in the claims, parts will be identified by specific names for convenience, but they are intended to be as generic in their application to similar parts as the art will permit.

Referring to the drawing, Figure 1 shows a length of stranded wire 10 covered with a braided sleeve 11 of synthetic resin fibres which can be softened and sealed by heat, such as cellulose acetate. Other fibres which may in some cases be used may be formed of nylon, vinyl resins and other materials which are heat fusible or heat softening. The covered wire used may be made of any length and may, for example, be taken from a reel as used.

In order to produce the sections of insulated wire desired, a heated instrument is brought into contact with the insulated sleeve 11 at spaced intervals along the length of the wire, the distance between the contact points corresponding to the length of insulating sleeve desired on the finished lead wire. As shown in Figure 2, for example, the wire is simply rolled along a heated rod or small heated soldering iron 12 which is at a temperature slightly above the softening temperature of the fibres of sleeve 11. The result of this procedure is to produce a bonded ring 13 around the wire at the point of contact with the heated instrument, the fibres at this point sticking together due to the heating. As an alternative to the method shown in Figure 2, the covered wire 10 may be clamped between a pair of heated jaws 14 and 15 of a clamping device to produce a melted ring about the wire.

The wire is then cut into sections of the desired length, the cuts being made through the wire and covering at approximately the middle of the points of fusion. Figure 4 illustrates a length of wire which has been cut through the points of fusion leaving one uncut fused ring at an intermediate point. This fused portion is quite brittle and the sleeve can readily be broken at this point by simply bending the wire back and forth between the fingers a few times thus separating the sleeve 11 into two sections. One of the sections may then be slid off the wire leaving the length of wire 10 with a sleeve section 11 covering part of its length only as shown in Figure 5. The sleeve 11, being quite elastic, may be

drawn back from the end of the wire leaving a bare end which can be attached to an electric terminal with or without tinning.

Where a bare section of wire is not required the wire may be cut as shown in Figure 6 at two fused points and the ends shoved back to expose free ends of the wire.

The fused ends of the sleeve are bonded together by the fusion and hence do not tend to fray out, as is the case where no bonding is obtained. This fraying has heretofore prevented the use of wire having braided sleeves without impregnating the sleeve with a binder. However, impregnation has given the braided covering too great a stiffness for many applications and hence it has not heretofore been possible in such applications to use braided coverings. Also it was somewhat of a problem heretofore to cut a sleeve at an intermediate point so as to provide a bare wire section as shown in Figure 5 without cutting through the wire. The brittleness of the covering at the fused sections provided by the present invention permits the sleeve to be readily broken at this point without the use of cutting tools and therefore greatly simplifies the stripping of the wire.

While the present invention, as to its objects and advantages, has been described herein as

carried out in specific embodiments thereof, it is not desired to be limited thereby but it is intended to cover the invention broadly within the spirit and scope of the appended claims.

5. What is claimed is:

1. The method of making insulated wire units from a length of wire insulated with a sheath formed of thermoplastic fibres which comprises heating the fibres in paths around said sheath at intervals along the length of said wire to form coalesced paths around said sheath, then cutting said wire and sheath at said paths to produce shorter lengths of wire having insulated sheaths thereon with the free ends thereof coalesced, and then pushing said free ends of said sheaths back to expose the ends of said shorter lengths of wire.

2. The method of making an insulated wire unit from a length of wire insulated with a sheath formed of thermoplastic fibres which comprises heating said fibres in a path around said sheath at an intermediate point along the length of said wire to coalesce said fibres at said point and produce a brittle point in said sheath, and then breaking said sheath at said brittle point and pushing the ends of said sheath thus formed back to expose a section of said wire.

ROBERT J. AUST.